

Dec. 20, 1966

P. A. STOWELL

3,293,059

ELECTROSTATIC IMAGE FIXING METHOD EMPLOYING INK AND  
RECORD MEDIUM HAVING CHEMICAL SIMILARITY

Filed Nov. 29, 1961

2 Sheets-Sheet 1



FIG. 1



FIG. 2

TO DRIVE MEANS

INVENTOR  
PHILIP A. STOWELL

BY

*Carl Fissell Jr.*  
AGENT

Dec. 20, 1966

P. A. STOWELL

3,293,059

ELECTROSTATIC IMAGE FIXING METHOD EMPLOYING INK AND  
RECORD MEDIUM HAVING CHEMICAL SIMILARITY

Filed Nov. 29, 1961

2 Sheets-Sheet 2



FIG. 3



FIG. 4



FIG. 5



FIG. 6



FIG. 7

INVENTOR  
PHILIP A. STOWELL

BY

Carl Fissell Jr.  
AGENT

# United States Patent Office

3,293,059

Patented Dec. 20, 1966

1

3,293,059

## ELECTROSTATIC IMAGE FIXING METHOD EMPLOYING INK AND RECORD MEDIUM HAVING CHEMICAL SIMILARITY

Philip A. Stowell, Paoli, Pa., assignor to Burroughs Corporation, Detroit, Mich., a corporation of Michigan

Filed Nov. 29, 1961, Ser. No. 155,712

1 Claim. (Cl. 117—17.5)

The present invention broadly relates to electrostatic printing and more particularly, although not necessarily exclusively, to a novel method and/or process for fixing electrostatically formed images onto recording material without the use of external applied heat. With still more particularity, the invention has to do with a method or process employing an electrostatic printing ink of a chemical formulation or group which demonstrates a natural chemical and mechanical affinity for a dielectric material bonded to or dispersed throughout a record medium or substrate, such for example; an electrostatic recording paper.

It is an object of the present invention to provide a method of fixing electrostatically formed images onto electrostatic record material without the use of externally applied heat.

It is another important object of the invention to provide a method of fixing electrostatically formed images onto electrostatic printing paper by means of pressure so as to cold weld or bond the ink to the paper.

In accordance with the foregoing objects and first briefly described herein, the present invention in the preferred and illustrated embodiment contemplates the employment of a resinous type ink and a resinous type dielectrically coated paper, both the ink and paper including one or more chemical compounds from a group of chemical compounds which have a natural affinity for one another such that when the latent image is formed on the printing medium and the medium is thereafter developed and made visible by the application of electrostatic ink thereto, the image may then be fixed by thereafter passing the paper through high pressure calendering apparatus whereby the ink is deformed and fused so as to chemically and mechanically bond it to the recording medium with which it has an affinity thus to provide a superior "copy" with sharper appearances, high color density, permanent and durable against adverse physical conditions such as abrasion, handling, folding etc.

With these and other objects in view, the invention consists in a novel method as will be more fully described and particularly pointed out in the appended specification and claim with reference to the accompanying drawings:

FIG. 1 is an elevational view, partially schematic, of a preferred form of apparatus embodying the present invention;

FIG. 2 is a view along the line 2—2 of FIG. 1 illustrating the pressure fixing assembly;

FIG. 3 is a sectional view along the line 3—3 of FIG. 1 illustrating a portion of the recording medium;

FIG. 4 is a plan view of a greatly enlarged portion of the recording medium with certain characters electrostatically recorded and fixed thereon according to the present method;

FIG. 5 is a greatly enlarged view along the line 5—5 of FIG. 4;

FIG. 6 is an enlarged view of one of the spots of FIG. 4 before fixing, and;

FIG. 7 is a similar view of the spots after fixing according to the invention.

Referring now to the figures of the drawings which will be discussed simultaneously in detail, there is seen a preferred embodiment of an electrostatic recording apparatus

2

10, including a supply reel 12 for a supply of recording material 14, such for example, as paper tape, prepared in accordance with the teachings hereinafter set forth. It is to be understood of course, that although the preferred embodiment of the invention is directed to a tape type printer, with certain modifications the same apparatus could be used for producing a continuous page of any desired width of printed copy. The present apparatus further includes a recording transducer 16 having a back-up anvil 18 adjustable by means 20 relative to the head 22, an electrostatic image developing member 24, and a pressure fixing mechanism 26.

The web of electrostatic recording paper 14, whose chemical composition will be described herein later on, is affixed to the reel 12 in conventional fashion, and is fed from the reel 12 over a roller 28 on a dancer arm 30 which is biased by spring 32 in a direction to apply suitable tension to the web. Thereafter the tape is fed over a guide roller 34 thence between the head 22 and the anvil 18. The anvil 18 is made adjustable so as to bring the paper into close proximity to the head 22 while causing the paper to bear upon the anvil over the full width and length thereof. The web is then fed around a roller 36 vertically downwardly to a second roller 38 and upwardly through a slot 40 into an ink container 42, the funnel shaped portion 44 of which is designed to contain a desired amount of finely particulated electrostatic recording ink 46, freely disposed thereon for gravity feed against the paper 14. Pressure guides 48 of felt, or similar material, provide a seal at the slot 40 to prevent accidental discharge of the ink into the surrounding atmosphere. The web is then fed across a beater mechanism 50 between a plurality of angled ink deflectors 52—52 to a doctor blade 54. Thereafter the paper 14 exits from the inker mechanism 24 and is fed between the rotating high pressure calendering rolls 56 and 58 of pressure fixer 26.

Roller 58 of the pressure fixer 26 is mounted on one end of a lever arm 60 which is pivoted by a pin 62 to the frame 64 of the apparatus 10. The opposite end of the lever arm 60 is biased vertically upwardly by means of a spring 66 and the adjustable shackle bolt 68 so that the pressure between the rollers 56 and 58 may be varied at will over a predetermined range. Thus, varying degrees of calendering pressure between the upper and the lower calendering rollers 56 and 58 may be provided. From the pressure fixer 26 the printed and fixed electrostatic image bearing material is fed to a container (not shown) e.g., take up reel, bin or bucket suitably disposed adjacent the exit portion thereof for containing the printed material until such time as it is to be used, i.e., viewed, etc.

Referring now to FIG. 5 wherein the electrostatic recording medium 14 is seen to comprise a cellulosic type base material, such for example, as paper 70 on which there has been coated a styreneated dielectric 72 which includes a polyvinylacetate and a polystyrene base. This material is substantially identical in formulation and composition to that described in copending U.S. application to P. A. Stowell, Serial No. 824,010, filed June 30, 1959, now Patent No. 3,097,964, and assigned to the same assignee as the present invention. This material has the desirable quality of remaining in colloidal suspension with many of the particles standing close to the surface of the coating material thus to form what is technically referred to as "tooth," i.e., a rough textured finish 74 with many minuscule projections thereon and may be produced in a manner set forth hereinafter. The aqueous or other vehicle may be alcohol or water with a fugitive base, e.g., ammonia. A polyvinylacetate copolymer (preferably a copolymer of vinyl acetate monomer with about 3% crotonic acid monomer) having carboxyl and hydroxyl groups on the polymeric molecules, the carboxyl groups being residual

radicals from the crotonic acid monomer and the hydroxyl groups coming from a small proportion of unesterified vinyl alcohol from the vinyl acetate monomer, the polymeric material being therefore dispersible in water containing free alkali and thus lyophilic, may be obtained under the trade name "Gelva" from Shawinigan Resins Corporation, 644 Monsanto Avenue, Springfield, Mass. In an aqueous solution of ammonium hydroxide having a pH from 8.7 to 9.5 there is dispersed colloidally, sufficient of such resin to produce a dispersion having, at room temperature, the viscosity of a moderately thin syrup. For Gelva type C-3-V-20, this requires a concentration of about twenty percent by weight of dispersion. Additional ammonium hydroxide must be added to adjust the pH to 8.5 to 8.7; it is presumed that the carboxyl groups are effective in promoting the dispersion of the resin, and that they cause the reduction of the pH; but this is merely a reasonable assumption. It has been found possible to render the final film opaque by dispersing, as by ball milling, in the dispersion of lyophilic resin, a pigment such as titanium dioxide sold commercially by the Titanium Pigments Company of New York City, New York, under the name "Titanox RA 50." A weight of such pigment equal to one-fourth the weight of the lyophilic resin sufficed to render the final film opaque. A mechanical dispersion of a different dielectric resin, which is insoluble and lyophobic in aqueous solutions, is prepared by ball milling in methanol for several hours a copolymer formed from styrene and alpha-methyl-styrene monomer having a melting point of about 112 degrees centigrade. The ball milling is continued until the average particle size of the copolymer is below one micron. The concentration of the ball milled dispersion is by weight about twenty-five percent of resin. To the colloidal ammoniacal dispersion of the polyvinylacetate copolymer there is added from three to six percent by weight of the ball milled methanol dispersion of polystyrene copolymer, mixing the two thoroughly. A polystyrene poly-alpha-methylstyrene copolymer satisfactory for this purpose is sold by the Pennsylvania Industrial Chemical Corporation, 120 State Street, Clairton, Pennsylvania, under the trade designation of "Piccotex-112." It should be observed particularly that the polyvinylacetate copolymer is insoluble in water, and non-hygroscopic; and in accordance with a common property of colloidal dispersions, a dispersion of this material suffers a rapid increase in viscosity upon a relatively small withdrawal of suspending liquid. The polystyrene (poly-alpha-methylstyrene) copolymer is reasonably hard, and sufficiently friable that it may readily be reduced in size by ball milling and has good dielectric properties.

The mixed colloidal and mechanical suspension whose preparation has already been described, is applied to a paper base 70, FIG. 5, by painting, rolling or dipping, or other coating techniques, with the following results: the paper absorbs the aqueous ammonia solution into its interior portion by capillary action, leaving at its surface a highly viscous colloid gel containing mechanically dispersed particles of polystyrene poly-alpha-methylstyrene copolymer. Upon drying, the gel deposits a continuous, flexible uniform thin film 72 of polyvinylacetate copolymer whose surface has what may be called tooth from the presence of the harder particles of polystyrene poly-alpha-methylstyrene copolymer, which render the surface capable of abrading the graphite of a pencil lead, and are believed to assist in the spreading of conventional writing ink over the surface, as was observed to occur. It is suspected that the hydrophilic carboxyl groups in the film render the film writable by fluid ink.

Experimental evidence demonstrates that when the resins in the dielectric 72 are compatible with, and chemically similar to, those in the ink 76, being used, (FIG. 6) molecular bonds can be established between the ink and the dielectric when the two are brought together under applied pressure. Thus, for ideal pressure fixing the ink 76 should comprise a thermoplastic resinous vehicle suitably

pigmented with carbon black so as to color the same as well as to provide a desired degree of electrical conductivity. At least a part of the resinous vehicle must include a resin which chemically is the same as or substantially similar to at least one of the resins which is a constituent of the dielectric 72 on the paper 70, earlier described herein. Presuming these conditions to be met, then when sufficient pressure is applied to the ink 76, FIG. 6, to press it against the dielectric and, due to the fact that the dielectric is sufficiently hard to support the ink, enough work is done on the ink to adiabatically increase its temperature to a level sufficient to cause it to soften slightly and to fuse and assume the shape of the particles 76', FIGS. 5 and 7, thereby welding or bonding itself to the similar resin in the dielectric 72. An example of an inking powder possessing the foregoing qualities and properties may be formulated as follows: 500 grams of Koppers Co. Dylex K85 is used as the binder for the ink. This material may be obtained from the Koppers Co., Inc. Plastics Division, 430 Park Avenue, New York 22, New York. K85 is a styrene-butadiene latex, 50% solids in water with a styrene-butadiene ratio of 80/20. To this is added 700 grams of Aquablak M, a dispersion of conductive furnace black in water, 50% solids made by Columbian Carbon Co., 380 Madison Avenue, New York 17, New York, and 300 grams of water. The resultant dispersion is spray dried in a Bowen Laboratory spray dryer, 240° maximum outlet temperature. The powder is sized by screening and elutriation (the latter as part of the drying process) to provide particles in the range of 16 to 100 microns.

The resinous ink particles 76 must have adequate hardness, however, so that a considerable amount of work must be done to deform them and at the same time they must not be excessively friable but must rather be capable of plastic deformation. In this way when high pressure is applied to them they will collapse, spread out slightly, FIGS. 6 and 7, and a comparatively large amount of work will be delivered to each particle with the result that such work will appear in the form of enough heat to fuse the particle. Thus the frictional work done by compressing the relatively hard ink particles acts to dissipate heat in, and thereby raise the temperature of, the ink particles before the heat can be transferred by conduction or otherwise to the paper coating and to the surroundings, so that the thermoplastic ink material softens and becomes molecularly bonded to the chemically similar material of the coating before there is any substantial removal of thermal energy from the ink particles. In the event that the dielectric has a very rough or toothed surface which is hard but there is no chemical similarity between its constituent resins and the constituent resins of the ink particles, then the ink particles may still be fused as predicted by the applied pressure and the resulting temperature increase but there apparently will be no molecular bonding between the ink and the surface of the dielectric. The ink 76 may nevertheless appear to be fairly well adhered because of being mechanically locked by being pressed into the interstices and the tooth on the surface of the dielectric. However, it is the combination of the mechanical bonding to a toothed dielectric surface and molecular bonding between the chemically similar and compatible resins in the pressure-fused ink and the dielectric surface which has been found to give "fixing" or ink-to-dielectric bonding, which is superior to either technique alone. Other examples of such chemically compatible resins include: polystyrene, polystyrene acrylonitrile, polystyrene butadiene and styrene-alpha-methylstyrene.

With the foregoing in mind it is seen that when the paper web 14 passes beneath the recording head 22 with the recording stylus, not shown, a latent image is produced upon the web which is thereafter made visible by passage of the web through the recording ink 46 as hereinabove set forth, thus to produce a visible image comprising a series 75 of dots 78 which while in and of themselves tending to

be fairly irregular in size, FIG. 4, are more or less made to appear uniformly regular due to the small size of the image relative to the comparatively large number of much smaller ink particles on each dot of the image and to the fact that the eye tends to desire the regular rather than irregular in its viewing of the image, FIG. 3. As now conditioned and made visible by the application of the electrostatic recording ink to the latent image each dot appears more or less as shown in FIG. 6, wherein the particles while substantially spherical are of varying size and are irregularly dispersed throughout the dot area. Thus it is seen in respect to FIG. 6, that there are voids between the particles comprising the dots as indicated by the reference character 80. These voids tend to reduce the contrast of the viewable image are relatively undesirable. It 15 is noted at this point that as is well known in the prior art, the voltages on the recording pins or stylus, generally speaking, control the dot size and also the separation between dots.

Thereafter as has been stated hereinabove, the web is 20 passed between the calendering rollers 56 and 58, whereupon, due to the extreme high pressure and adiabatic heating as hereinbefore mentioned, the individual ink particles 76 in each of the dots 78 are heated and fused tending to deform and flow together slightly to form a 25 dot 78' of the type seen in FIG. 7, wherein the majority of the voids 80 are missing as a result of the fact that the adjacent contiguous areas between the dots are filled up due to the aforementioned flowability. Thus an extremely high contrast image is produced having much better 30 definition than heretofore was obtainable with the known prior art electrostatic fixing techniques.

There is thus described a method of electrostatic recording wherein a recording medium such as paper is provided with a dielectric material which is sufficiently hard to cause somewhat thermoplastic recording ink particles to deform under calendering pressure without shattering or embedding themselves in the dielectric surface thereby enabling the ink firmly to adhere to the recording material effectively pressure welding and molecularly bonding the resin of the ink to the dielectric of the paper. A certain mechanical interlocking with the resin ink also occurs as the pressure forces the ink to conform intimately with the surface contours of the dielectric. This further enhances the bond between the ink and the dielectric. 35 40

What is claimed is:

The method of fixing a latent electrostatic image without the use of externally applied heat comprising the steps of:

- 5 (a) providing an electrostatic record medium with a dielectric thin film coating of styrenated resin material whereby to provide a toothed or textured surface thereupon,
- (b) preparing a particulate electrostatic recording ink with a styrenated resin material having a characteristic and chemical similarity to the styrenated textured surface forming material in the record medium, and being sufficiently softer than this material whereby the ink particles will be deformed by the latter upon pressure contact therewith,
- (c) producing a latent electrostatic image of the desired information upon the dielectric surface of said record medium,
- (d) applying said recording ink to said dielectric surface thus to produce a visible image of said information, and
- (e) finally permanently fixing said ink to said record member by passing said record member between adjustable calendering rolls so as to vary the amount of the calendering pressure upon said record member whereby said ink is deformed and adiabatically heated such that the ink particles are caused to collapse slightly raising their temperatures and fusing the same substantially eliminating any voids therebetween and chemically and mechanically bonding the ink to the textured surface of the dielectric material effectively permanently affixing the image on said record member.

#### References Cited by the Examiner

##### UNITED STATES PATENTS

|           |         |                |       |          |
|-----------|---------|----------------|-------|----------|
| 2,944,147 | 7/1960  | Bolton         | ----- | 346—74   |
| 3,012,839 | 12/1961 | Epstein et al. | ----- | 346—74   |
| 3,094,429 | 6/1963  | Howell         | ----- | 117—17.5 |

BERNARD KONICK, Primary Examiner.

IRVING SRAGOW, Examiner.

45 P. F. ROTH, R. M. JENNINGS, Assistant Examiners.